

## UNITED STATES PATENT OFFICE

2,196,630

PROCESS OF PRODUCING SOFT LUSTER  
ARTIFICIAL SILKAugust Hartmann, Berlin-Lichterfelde, Germany,  
assignor to American Bemberg Corporation,  
New York, N. Y., a corporation of DelawareNo Drawing. Application June 5, 1935, Serial  
No. 25,129. Renewed August 26, 1939. In  
Germany June 22, 1934

7 Claims. (Cl. 18—54)

The present invention relates to a process of producing soft-luster products, such as artificial silk, from cuprammonium cellulose solutions.

The primary object of this invention has to do with the spinning of cuprammonium cellulose solutions into funnels without the assistance of special delustering agents, and without a delustering after-treatment of the finished, artificial silk.

Another object of this invention relates to the formation of a brittle surface skin on a cellulose filament or yarn which, subsequently, is ruptured by stretching in the funnel.

A third object of this invention has to do with the addition of a predetermined amount of an acid substance, such as an acid or an ammonium salt, to the washwater, circulating in the funnel, to form soft-luster cuprammonium cellulose products.

Other objects of this invention will become apparent to those skilled in the art from a study of the following specification.

It has been found by experimentation that soft-luster filaments and yarns can be produced from cuprammonium cellulose solutions by admixing such an amount of an acid substance to the precipitating water that the freshly precipitated cellulose has still an alkaline reaction upon leaving the spinning funnel and not an acid one. It has, furthermore, been found that it becomes impossible to form continuous filaments or threads when the acid in the precipitating water is increased to such extent that the cellulose, issuing from the funnel, acquires a neutral or acid reaction. For this reason, the present invention is limited to such acid precipitating solutions which allow the formation of slightly alkaline products under stretching in a funnel containing such solutions. Any suitable ammonium salt or

acid, such as sulphuric, tartaric, oxalic, acetic, citric, formic acid, etc., may be used in combination with water provided its amount is regulated, as set forth above. The optimum, minimum and maximum amount of the acid substance to be added to a given amount of water must be varied, since it depends upon a number of factors, such as the composition of the cuprammonium cellulose solution per se, the speed of spinning, the purity and temperature of the precipitating solution in the funnel, etc. By using, for example, a cuprammonium cellulose solution containing about 8% of cellulose, 8% of ammonium hydroxide, and 3% of copper, and spinning it to a thickness of 120 deniers at a speed of 30 meters

per minute with a water consumption of about 600 cc. per minute (30° C.), the maximum addition of sulphuric acid, for example, is about 4 grams per liter of precipitating water. The addition of about 3 grams of sulphuric acid to one liter of water still allows the formation of slightly alkaline filaments and threads, although the precipitating (funnel) water has an acid reaction. In this manner, soft-luster cellulosic products can be produced in the form of continuous filaments, 10 yarns, etc.

The precipitating water, as stated above, may contain an acid compound, i. e., an inorganic or organic acid or an ammonium compound, which does not deleteriously affect the precipitated cellulose during the formation and rupturing of its brittle surface skin by stretching the cellulosic product in said precipitating water. Although the aforementioned ammonium compounds assist in coagulating the cellulose and allow the formation per se of soft-luster products when being present in the precipitating water, they do not create the same effect as the equivalent amount of a free acid. Thus, it has been found that the addition of an acid in combination with an ammonium compound to the precipitating water may be larger than that one of a free acid, part of which having been replaced by an ammonium compound in stoichiometrical proportion. For this reason, it is possible to spin successfully cuprammonium cellulose solutions in a precipitating water containing about 2 grams of sulphuric acid and 3 to 4 grams of ammonium sulphate, although these solutions cannot be spun in water containing more than 4 grams of free sulphuric acid per liter. The maximum addition of ammonium sulphate is about 5 grams per liter of water containing about 2 grams of sulphuric acid.

Special advantages are obtained by using the precipitating solutions, set forth above, in combination with the so-called "circulation process." In this process, in which a considerable amount of the precipitating solution is tapped from the bottom of the funnel and recirculated to its top portion, troubles are experienced with alkaline precipitating water since it causes the precipitation of difficultly filtrable, basic copper salts. These troubles, however, are eliminated by using and recirculating acid precipitating water in accordance with my present invention. In this manner the conventional "circulation process" is simplified and rendered more efficient, and sometimes it becomes even unnecessary to use softened

water, obtained with the assistance of permutite, etc., since the unfavorable effect of calcium bicarbonate can be eliminated by the addition of small amounts of an acid to hard water.

5

*Example*

A cuprammonium cellulose solution, containing about 8% of cellulose, 8% of ammonium hydroxide and 3% of copper, is spun in a funnel in accordance with the conventional stretch-spinning process under the following conditions:

10 Total titre \_\_\_\_\_ deniers 120  
Spinning speed per minute \_\_\_\_\_ meters 30  
15 Water consumption per minute \_\_\_\_\_ cc 600  
Temperature of precipitating solution  $^{\circ}$  C 30

20 The aqueous precipitating water contains about 3 grams of sulphuric acid per liter of water (soft water obtained with permutite). The filaments and yarns obtained are of soft-luster.

25 Modifications of the present invention will be readily recognized by those skilled in the art, and it is desired to include all modifications coming within the scope of the appended claims.

What is claimed is:

1. In the process of producing soft-luster products, the step which comprises spinning a cuprammonium cellulose solution under stretching in a funnel containing water and an acid to precipitate cellulose therein, said acid being present in said water in such an amount that the precipitated cellulose remains slightly alkaline upon leaving said funnel.

30 2. In the process of producing soft-luster products, the step which comprises spinning a cuprammonium cellulose solution under stretching in a funnel containing hard water and an acid to precipitate cellulose therein, said acid being present in said water in such an amount

40

that the precipitated cellulose remains slightly alkaline upon leaving said funnel.

3. In the process of producing soft-luster products, the step which comprises spinning a cuprammonium solution under stretching in water containing about 2 to 4 grams of sulphuric acid per liter.

4. In the process of producing soft-luster products, the step which comprises spinning a cuprammonium cellulose solution containing about 8% cellulose, 8% of ammonium hydroxide and 3% of copper under stretching in a funnel containing water and about 0.2% of sulphuric acid, said cellulose solution being spun at a speed of about 30 meters per minute.

15 5. In the process of producing soft-luster products, the step which comprises spinning a cuprammonium cellulose solution under stretching in a funnel containing water, an acid and an acid compound to precipitate cellulose therein, said acid and acid compound being present in said water in such an amount that the precipitated cellulose remains slightly alkaline upon leaving said funnel.

20 6. In the process of producing soft-luster products, the step which comprises spinning a cuprammonium cellulose solution under stretching in a funnel containing hard water, an acid and an acid compound to precipitate cellulose therein, said acid and acid compound being present in said water in such an amount that the precipitated cellulose remains slightly alkaline upon leaving said funnel.

25 7. In the process of producing soft-luster products, the step which comprises spinning a cuprammonium cellulose solution under stretching in a funnel containing water, about 0.2% of sulphuric acid and about 0.3 to 0.5% of ammonium sulphate.

AUGUST HARTMANN. 40